

No. 756,223.

PATENTED APR. 5, 1904.

E. FAHRIG.

## PROCESS OF TREATING LOW GRADE ORES AND TAILINGS BY ELECTROLYSIS.

APPLICATION FILED MAY 9, 1903.

**NO MODEL.**



Witnesses  
Henry J. Schubert.  
John J. Little

By his Attorney, *Ernst Fahrig*  
*James Niles*

## UNITED STATES PATENT OFFICE.

ERNST FAHRIG, OF PHILADELPHIA, PENNSYLVANIA.

## PROCESS OF TREATING LOW-GRADE ORES AND TAILINGS BY ELECTROLYSIS.

SPECIFICATION forming part of Letters Patent No. 756,223, dated April 5, 1904.

Application filed May 9, 1903. Serial No. 156,392. (No specimens.)

*To all whom it may concern:*

Be it known that I, ERNST FAHRIG, a citizen of the United States, residing in Philadelphia, in the county of Philadelphia and State of 5 Pennsylvania, have invented certain new and useful Improvements in Processes of Treating Low-Grade Ores and Tailings by Electrolysis, of which the following is a specification.

This invention relates to an improved process of treating low-grade ore and tailings containing a low percentage of precious metals, so that the same can be worked up effectively by electrolysis.

In many mines heretofore abandoned owing 15 to the low percentage of gold and silver contained in the ores it is possible to work up the same, also the accumulated tailings of abandoned mines, by my improved process, as the same is adapted to regain almost every trace 20 of precious metal contained in the ores and tailings in a successful manner and at a low expense, giving a yield of metal which compensates for the cost of installation and operation.

25 For this purpose the invention consists of a process of treating low-grade ores and tailings by electrolysis by conducting a mixture of the finely-ground ores or tailings, water, and a suitable electrolyte forming a pulp by 30 gravity alternately into contact with inclined cathode and anode plates, collecting the deposited film of precious metals by scraping the same from said cathode-plates, subjecting the ores or tailings after this electrolytic extraction to an oxidizing and leaching action, and finally subjecting them to an electrolytic separation by precipitation, as will be fully 35 described hereinafter and finally pointed out in the claims.

40 The accompanying drawing represents an apparatus for carrying out my improved process of treating low-grade ores and tailings by electrolysis, part in vertical section and part in side elevation.

45 In carrying out my improved process the ore and tailings are crushed to any desired mesh above 20<sup>2</sup> and are then conducted to an elevator E and dumped by the same into a charging-vat A. To the charging-vat A a 50 suitable electrolyte is added, and water is ad-

mitted by a supply-pipe a, having a valve a', that passes through the bottom of the vat until the quantity of water and electrolyte admitted amounts to about sixty per cent. of the weight of the dry ore or tailings, which produces a pulp sufficiently liquid to flow through the pipe C, which is connected with the circulating-pump P, that is located below the charging-vat A and which serves to lift the pulp from the vat A through a stand-pipe C to the upper end 60 of a tower T. The tower T is made of square or rectangular shape, according to the capacity required. The frame of the tower is suitably held together by stay-pieces separated by about three feet from each other. The 65 tower is provided with two doors that extend the full length of the same and are hinged to the side walls of the tower-frame. In the interior of the tower T are arranged, at equal distances from each other, metal grooves m for the 70 reception of the cathode-plates D. The lower ends d of the cathode-plates D are turned up so as to form a rim of about one-quarter of an inch in height. The cathode-plates D extend from one wall to near the opposite wall and leave 75 sufficient space to permit that amount of liquid pulp to pass readily over the cathode-plates and between the same and the opposite wall corresponding to the capacity of the pipe C. The edge of the cathode-plates is 80 even with the edge of the frame, so that when the doors are closed suitable contact-springs on the doors, which are connected with one pole of the dynamo, form a reliable contact with the inclined cathode-plates. When opening the doors, the cathodes can be readily removed from the tower by sliding them out of their grooved guideways for stripping or scraping off the deposit on the same. The 85 cathodes D are made of sheet-copper or other suitable metal of sufficient thickness and strength for resisting the volume and pressure of the pulp passing over the same for treatment. Below each cathode is arranged an inclined anode B, which is made of graphite or 90 other suitable material and securely attached to the frames of the side walls or to the doors of the tower. The anodes are connected with the opposite pole of the dynamo. A dynamo 95 G of low voltage and ample amperage is suit- 100

ably connected with a switchboard H, which is provided with a rheostat or regulator R, a voltmeter V, ammeter M, and a main switch S and complete the necessary electrolytic apparatus. The voltage is approximately five to seven volts, and the amperage corresponds to 0.08 to 0.1 ampere per square foot of cathode. However, I do not wish to confine myself thereto, as it depends on the constituency and character of the ore under treatment. For the electrolytic precipitation of precious metals from solution I prefer two to five volts and from 0.05 to 0.06 ampere per square foot of cathode-plate.

15 In the charging-vat A is arranged a mercury-trap N, into which the pulp is discharged from the chute D' below the lowermost cathode-plate D of the tower T until it overflows from and runs into the charging-vat A. The 20 electrolyzing action is kept up in the tower for about one hour per ton of ore charged. The electrolyzing action is due to the oxidation of the quickened surface of the cathode-plates, as the nascent hydrogen constantly escaping from the pulp during the passage of the same through the tower has a tendency to quicken the cathode-plates, and thus keep the amalgam in a condition to easily retain any precious metal which might be in the pulp. 25 Moreover, the electromotive force by virtue of the nascent hydrogen, chlorin, and oxygen, as the case may be, according to the character of the electrolyte used, decomposes the particles of metal in the mineral-containing earthy matter and gangue, so that the precious-metal particles are brightened, and thus prepared to be either retained by amalgamation or to be brought by the continued action of the active electrolyte under a suitable elec- 30 tromotive force into solution.

The stand-pipe C' is connected by a valved branch pipe C<sup>2</sup> with an inclined riffle-trough F, which is made of suitable length and provided at its bottom with transverse riffles f 40 equidistant from each other for catching any heavy or coarse material, iron pyrites, or concentrates, so that the clear pulp can pass over the riffles f and into a leaching-tank L. This tank is gradually filled with the different 45 charges obtained from the charging-vat A after the precious metal contained in the same has been partially extracted by the electrolytic action of the tower. When the tank L is filled, the pulp or ore, water, and electrolyte mixture feeding into the vat A is interrupted and the liquid flows through pipe h, provided with a valve b, to the vat A, through the tower T, over the riffle-trough F, back to the leaching-tank L. This is continued until 50 tests taken from time to time show that the precious metals have been sufficiently extracted by the electric current.

It has been found by practical tests that from twelve to eighteen hours of electrolyzing and oxidizing is sufficient for leaving the 55

pulp in the leaching-tank for about from ten to twelve hours, after which the liquid, still containing some metal, may be drawn off by decantation or other suitable means and either run through a filter-press or the precious metal still contained therein recovered by subjecting it again to electrolytic precipitation or any well-known method—as, for instance, to the action of a large battery—in which the traces of precious metal still contained in the leached mass may be extracted, while the remaining portion is run off as waste.

The riffle-trough F, over which the extracted pulp is passed, has the double object of agitating the pulp and thoroughly oxidizing it 80 while passing over the riffles f in the riffle-trough. A set of blow-pipes is connected with each vat and riffle-trough for a still more thorough oxidizing of the pulp.

The electrolyte employed may be any oxy 85 chlorid or chlorids, or a weak solution of potassium cyanid or hypochlorid, or any other electrolyte may be used.

My improved process of treating low-grade ores or tailings is carried on as follows: The 90 ore is mixed in the charging-vat A with a suitable quantity of water and a suitable electrolyte, as any oxychlorid or chlorid, or a weak solution of potassium cyanid or hypochlorid, which mixture forms a pulp which is 95 pumped up through the stand-pipe to the hopper-shaped upper end T' of the electrolytic tower T, in which it traverses alternately between a pair of cathode-plates D and anode-plates B and is thus subjected to the electrolytic action of the current. The precious metals are deposited on the cathode-plates D, which are removed from time to time from the tower and scraped or stripped. The cathodes and anodes are so arranged in their relative positions that the pulp under a pressure corresponding to a section of the side of the tower is forced to make contact between the under surface of the anode and the upper surface of the cathode plates. The partially-extracted pulp passes from the lower end of the tower T into the mercury-trap N and overflows in the charging-vat A, from which it is lifted again by the stand-pipe C', this treatment being kept up for about an hour 105 per ton of ore charged. After the greater quantity of precious metals in the pulp are deposited by the electrolytic action the two-way valve C<sup>2</sup> is turned and the partially-extracted pulp of the vat A caused to pass over the riffles f of the riffle-trough F into the leaching-tank L. The process of charging the tank A, subjecting the pulp to electrolytic action, and discharging the charge of partially-extracted pulp onto and over the riffle-trough 110 F and into the leaching-tank L is repeated until the capacity of the leaching-tank is reached. The pulp which has been subjected to this process is permitted to stand in the leaching-tank for some time, whereupon it is 115 120 125 130

returned to the charging-vat A, passed again through the tower T, over the riffles f of the riffle-trough F, until the tests show that the metals contained therein are sufficiently extracted by the electrolytic action of the current. Finally, the partially-extracted pulp is subjected to filtration or decantation to regain from the filtered or decanted liquor the precious metal in solution. The liquor is heated to 120° or 130° Fahrenheit and then subjected, preferably by steam, to electrolysis in an electrical depositing or precipitation battery, or both, also charged from the dynamo. The pulp, after a second washing for the last trace of precious metal in solution, is run off as waste.

The tower action and the automatic action from beginning to end enables a large amount of work to be done with the least possible manual labor, while the tower action, in which the repeated rise and fall of pulp takes place through a space filled with an oxidizing atmosphere at a pressure equal to the height of the tower, has an extraordinary effect on the ore under treatment.

The use of my improved process will cause the reworking of mines which are now abandoned, as the amount of precious metals obtained thereby compensates for the cost of installation and operation in a short time.

Having thus described my invention, I claim as new and desire to secure by Letters Patent—

1. The process herein described of treating low-grade ores and tailings by electrolysis for regaining the precious metals contained in the same, which consists in grinding the ore or tailings, then mixing the same with a suitable quantity of water and a suitable electrolyte so as to form a pulp, passing said pulp by gravity between a series of pairs of inclined anode and cathode plates arranged tower fashion one below the other, and removing from time to time the precious metal deposited on said cathode-plates, substantially as set forth.

2. The process herein described of treating low-grade ores and tailings by electrolysis, which consists in subjecting a pulp of ore or tailings, water and a suitable electrolyte to an electrolytic action by passing the same by gravity between alternately-inclined pairs of anode and cathode plates arranged in a tower one below the other so as to deposit the precious metals on the cathode-plates, subjecting the partially-extracted pulp to an oxidizing action, and then to a leaching action, and finally to a second electrolytic action for removing the remaining traces of precious metal, substantially as set forth.

3. The process herein described of treating low-grade ores and tailings by electrolysis,

which consists in subjecting a pulp of ore or tailings, water and a suitable electrolyte to an electrolytic action by passing the same between a plurality of pairs of inclined anode and cathode plates arranged in a tower one 65 below the other for depositing the precious metals thereon, subjecting the partially-extracted pulp to an oxidizing action, then to a leaching action for some time, and then to a successive electrolytic, oxidizing and leaching action, until the precious metals in the partially-extracted pulp have been almost completely dissociated, dissolved and gone into solution, and finally to the electrolytic action of a battery for obtaining the remaining traces 70 of the precious metal, substantially as set forth.

4. The process herein described of treating low-grade ores and tailings by electrolysis, which consists in subjecting a pulp of ore or tailings, water and a suitable electrolyte to an electrolytic action by passing the same between a plurality of pairs of alternately-inclined anode and cathode plates arranged in a tower one below the other for depositing the 80 precious metals thereon, subjecting the partially-extracted pulp to an oxidizing action, then to a leaching action for some time, then to a successive electrolytic, oxidizing and leaching action, until the precious metals have 85 been almost completely dissociated, dissolved and gone into solution, then subjecting the same to defecation, heating the defecated liquor, and finally subjecting the liquor to an electrolytic action, substantially as set forth. 90

5. The process herein described of treating low-grade ores and tailings by electrolysis, which consists in repeatedly passing a mixture of ground ore or tailings, water and a suitable electrolyte between a series of pairs of alternately - inclined anode and cathode plates arranged tower fashion one below the other, substantially as set forth.

6. The process herein described of treating low-grade ores and tailings by electrolysis, which consists in passing a mixture of ground ore or tailings, water and a suitable electrolyte between a series of pairs of alternately-inclined anode and cathode plates arranged tower fashion one below the other in an oxidizing atmosphere at a pressure equal to the height of the tower, substantially as set forth.

In testimony that I claim the foregoing as my invention I have signed my name in presence of two subscribing witnesses.

ERNST FAHRIG.

Witnesses:

PAUL GOEPEL,  
C. P. GOEPEL.